# EUROPEAN PATENT SPECIFICATION

(11) **EP 3 357 595 B1**
(45) Date of publication and mention of the grant of the patent: **19.05.2021**
(21) Application number: 16850846.3
(22) Date of filing: 28.07.2016
(51) Int. Cl.: B21B 25/00, C23C 4/08

(54) **PLUG AND METHOD FOR MANUFACTURING SAME**
STECKER UND VERFAHREN ZUR HERSTELLUNG DAVON
POINÇON ET SON PROCÉDÉ DE FABRICATION

(30) Priority: 28.09.2015 JP 2015190400
(43) Date of publication of application: 08.08.2018
(73) Proprietor: Nippon Steel Corporation, Tokyo 100-8071 (JP)
(72) Inventor: HIGASHIDA, Yasuto, Tokyo 100-8071 (JP); HIDAKA, Yasuyoshi, Tokyo 100-8071 (JP)
(74) Representative: Zimmermann & Partner Patentanwälte mbB
(86) International application number: PCT/JP2016/072212
(87) International publication number: WO 2017/056669

(56) References cited:
- EP-A1- 2 845 657
- WO-A1-2014/013963
- JP-A- H08 193 241
- JP-A- 2013 226 565

## Description

### TECHNICAL FIELD

The present disclosure relates to a plug, and more particularly, to a plug used to pierce a billet and a method of manufacturing the same.

### BACKGROUND ART

The Mannesmann pipe-making method is widely used to manufacture seamless pipes. The Mannesmann pipe-making method involves heating a billet to a predetermined temperature and using a piercing mill to perform piercing/rolling on the billet. The piercing mill includes a pair of skewed rolls and a plug. The plug is positioned on a pass line between the skewed rolls. The piercing mill uses the skewed rolls to rotate the billet in a circumferential direction and, at the same time, pushes it against the plug to perform piercing/rolling on the billet, thereby producing a hollow shell.

In the case of a conventional plug, a coating of oxidized scale is formed on the surface of the base material before the piercing/rolling of a billet. The coating of oxidized scale is formed by performing heat treatment on the plug. This provides sufficient heat insulation, lubricity and seizure resistance of the surface of the plug.

The coating of oxidized scale gradually wears off due to repeated piercing/rolling. The coating wears off each time piercing/rolling is performed (i.e. for each pass). When part of the coating is completely worn off and lost, part of the base material of the plug is exposed. Then, exposed portions of the base material may be eroded or the plug may seize on the billet, i.e. opposite material, at which point the life of the plug expires.

Particularly, the coating of oxidized scale wears off significantly when billets made of stainless steel are pierced, leading to a very short life for the plug. When billets made of stainless steel are pierced, the coating usually wears out in several passes. Each time a coating wears out, a heat treatment is necessary to produce an oxidized scale on the surface of the base material of the plug. The heat treatment typically requires several hours to several tens of hours. Thus, the efficiency with which a coating of oxidized scale is formed is low.

To address this, Japanese Patent No. 4279350 proposes forming a coating made of iron and iron oxides on the surface of the base material of the plug by electric-arc spraying. According to Japanese Patent No. 4279350, the coating is made from iron wire only, and the time required to form the coating is several minutes to several tens of minutes, which is relatively short. This enables forming a coating on the surface of the base material at low costs and with high efficiency. The sprayed coating has a higher adhesion with respect to the base material and a higher wear resistance than a coating of oxidized scale. This increases the life of the plug.

JP 2013-248619 A discloses forming a sprayed coating containing iron and iron oxides on the surface of the base material of the plug before performing heat treatment on the plug.

WO 2014/013963 discloses forming, on the surface of the base material of the plug, an Ni-Cr layer that serves as a foundation for a sprayed coating containing iron and iron oxides.

JP S61(1986)-286077 A discloses forming a coating on the surface of a mandrel for a rolling mill for steel pipes by spraying metal-based powder, before performing hot isotropic pressurization on the mandrel.

JP H05(1993)-36502 A and JP H03(1991)-125076 A each disclose a method of forming a sprayed coating, although not applied to a plug used for piercing a billet. JP H05(1993)-36502 A discloses forming a sprayed coating of ultrahard alloy on the surface of a base and forming a plated coating of an Ni-P alloy on the sprayed coating before performing hot isostatic pressing on the base. JP H03(1991)-125076 A discloses spraying a wear-resistant material on the surface of a base before performing a sealing treatment thereon by spraying a powder material capable of closing pores, and performing hot isostatic pressing on the base. The preamble of claim 1 is based on JP H08 193241 A.

### DISCLOSURE OF THE INVENTION

A coating formed by arc spraying of iron wire (or steel wire) has a high adhesion with respect to the base material of the plug and a high wear resistance, which increases the life for the plug. However, for example, when a billet with high strength made of a high alloy is to be pierced or when the pierced length of the billet is extremely long, part of the coating may peel off the surface of the base material during piercing. If part of the base material is exposed as a result of the peeling of the coating, the plug may be eroded or the billet may seize on the plug, with the exposed portions working as initiation points.

An object of the present disclosure is to provide a plug that achieves prevention of peel-off of the coating, and a method of manufacturing such a plug.

A plug according to the invention is defined in claim 1.

The present invention is also directed to a method according to claim 8 of manufacturing a plug according to claim 1. The plug is used for piercing a billet. The method includes: preparing a plug body; forming a body coating on a surface of the plug body by performing arc spraying using iron wire; and forming a surface-layer coating on the body coating by performing arc spraying using iron wire at a spray distance shorter than that at completion of the formation of the body coating.

The plug according to the present disclosure and the method of manufacturing it achieve prevention of peel-off of the coating.

### BRIEF DESCRIPTION OF THE DRAWINGS

[FIG. 1] FIG. 1 is a partial cross-sectional view of a plug according to an embodiment.
[FIG. 2] FIG. 2 is an enlarged view of portion II of the plug shown in FIG. 1.
[FIG. 3] FIG. 3 is an example of a microscopic image of a cross section of the coating.
[FIG. 4] FIG. 4 is a brightness histogram for the microscopic image shown in FIG. 3.
[FIG. 5] FIG. 5 is a brightness histogram for the microscopic image shown in FIG. 3, illustrating how to express the microscopic image using three values.
[FIG. 6] FIG. 6 is a three-value image derived from the microscopic image shown in FIG. 3.
[FIG. 7] FIG. 7 illustrates a method of manufacturing the plug shown in FIG. 1.
[FIG. 8] FIG. 8 is a graph showing the relationship between the spray distance during coating formation and the porosity of the coating.
[FIG. 9] FIG. 9 is a graph showing the relationship between the spray distance during coating formation and the content of oxides in the coating.
[FIG. 10] FIG. 10 is a graph showing the relationship between the spray distance during coating formation and the tensile strength of the coating.
[FIG. 11A] FIG. 11A illustrates the effects of the plug according to the embodiment.
[FIG. 11B] FIG. 11B illustrates the effects of the plug according to the embodiment.
[FIG. 12A] FIG. 12A illustrates the mechanism through which the coating of a conventional plug peels off.
[FIG. 12B] FIG. 12B illustrates the mechanism through which the coating of a conventional plug peels off.
[FIG. 12C] FIG. 12C illustrates the mechanism through which the coating of a conventional plug peels off.
[FIG. 12D] FIG. 12D illustrates the mechanism through which the coating of a conventional plug peels off.

### EMBODIMENTS FOR CARRYING OUT THE INVENTION

The present inventors did extensive research and found out the mechanism through which the coating of a plug that is piercing a billet peels off. FIGS. 12A to 12D illustrate the mechanism through which the coating of a conventional plug peels off. FIGS. 12A to 12D each schematically show a cross section of the plug near its surface.

As shown in FIG. 12A, before the piercing of a billet, a coating 102 is present on the surface of the plug body 101. The coating 102 includes pores 103.

As shown in FIG. 12B, when the piercing of the billet begins, the friction between the coating 102 and billet causes a load in a direction along the surface of the coating (i.e. shear direction) to act on the coating. This deforms the coating 102, producing cracks C on the surface of the coating 102, with the deformed portions working as initiation points.

As shown in FIG. 12C, the load in the shear direction acting on the coating 102 causes cracks C to progress along the interface between the plug body 101 and coating 102. As a result, part of the coating 102 peels off, as shown in FIG. 12D.

It occurred to the present inventors that the peel-off of the coating may be prevented by preventing deformation and cracking of the coating during the piercing of the billet. The present inventors did further research and completed the plug according to the embodiment and the method of manufacturing it.

A plug according to an embodiment is used for piercing a billet. The plug includes a plug body, a body coating, and a surface-layer coating. The body coating is provided on a surface of the plug body. The body coating contains iron and iron oxides. The surface-layer coating is provided on the body coating. The surface-layer coating contains iron and iron oxides. The surface-layer coating has a porosity lower than that of a region of the body coating adjacent to the surface-layer coating and having a thickness equal to that of the surface-layer coating (first arrangement).

In the first arrangement, on the body coating provided on the surface of the plug body is further provided a surface-layer coating. The surface-layer coating has a porosity that is lower than that of a region of the body coating that is located adjacent to the surface-layer coating. Thus, the surface-layer coating is denser and has a higher strength than the body coating. This will prevent the surface-layer coating and the body coating covered with the surface-layer coating from deforming due to the load in the shear direction, thereby preventing deformation-derived cracks. As a result, the coatings will be prevented from peeling off the surface of the plug body.

The porosity of the surface-layer coating may be not higher than 2.5 % (second arrangement).

In the second arrangement, the porosity of the surface-layer coating is low enough to provide a denser surface-layer coating with higher strength. This will further prevent deformation and cracking of the coatings, thereby preventing peel-off of the coatings more reliably.

The thickness of the surface-layer coating may be not larger than 250 µm (third arrangement).

In the third arrangement, the thickness of the surface-layer coating is small enough to improve heat removal from the surface-layer coating. This will reduce the temperature increase in the surface-layer coating during piercing, thereby preventing the billet from seizing on the plug.

A method of manufacturing a plug according to an embodiment includes: preparing a plug body; forming a body coating on a surface of the plug body by performing arc spraying using iron wire; and forming a surface-layer coating on the body coating by performing arc spraying using iron wire at a spray distance shorter than that at completion of the formation of the body coating (fourth arrangement).

In the fourth arrangement, the surface-layer coating is formed by, after the formation of the body coating, performing arc spraying with reduced spray distance. This will reduce the porosity of the surface-layer coating to be lower than the porosity of a region of the body coating adjacent to the surface-layer coating such that the body coating will be covered with a surface-layer coating that is dense and has a high strength. This will prevent the coatings from deforming due to the load in the shear direction during piercing, thereby preventing deformation-derived cracking. As a result, the coatings will be prevented from peeling off the surface of the plug surface.

Further, in the fourth arrangement, both the body coating and surface-layer coating are formed by arc spraying of iron wire. That is, the body coating and surface-layer coating are formed from the same material and with the same technique. This will enable successively forming the body coating and surface-layer coating within the same step. This will facilitate producing a plug with a body coating and a surface-layer coating.

The forming the body coating may perform arc spraying while the spray distance is gradually increased (fifth arrangement).

For arc spraying, increased spray distance results in increased content of oxides in the coating. In the fifth arrangement, the spray distance used to form a region of the body coating adjacent to the plug body is relatively small. Thus, the region adjacent to the plug body has a high iron content and a low oxide content. This will improve the adhesion of the body coating with respect to the plug body. On the other hand, the spray distance used to form a region of the body coating adjacent to the surface-layer coating is relatively large. Thus, the region adjacent to the surface-layer coating has a high oxide content, which reduces heat conductivity. This will improve the heat insulation of the body coating, thereby preventing the billet from seizing on the plug.

Embodiments will now be described in detail with reference to the drawings. The same and corresponding elements in the drawings are labeled with the same characters and their description will not be repeated. For convenience of explanation, elements may be simplified or shown schematically in the drawings, and some elements may not be shown.

### [Construction of Plug]

First, the construction of the plug will be described. As shown in FIG. 1, a plug 10 according to an embodiment includes a plug body 1, a body coating 2, and a surface-layer coating 3. FIG. 1 shows a cross section of the plug 10.

The plug body 1 has a circular transverse section with an outer diameter that increases as it goes from the tip of the plug body 1 toward its rear end. In short, the plug body 1 is generally shaped like a projectile.

The body coating 2 is formed on the surface of the plug body 1. The body coating 2 covers the entire surface of the plug body 1 except for the rear end surface of the plug body 1. The thickness of the body coating 2 may not be constant over the entire plug. For example, the portions of the body coating 2 that are located on the tip portion 11 of the plug body 1 have larger thicknesses than the portions located on the trunk portion 12 of the plug body 1.

The surface-layer coating 3 is formed on the body coating 2. The surface-layer coating 3 covers the entire the body coating 2. The thickness of the surface-layer coating 3 is smaller than the thickness of the body coating 2. The thickness of the surface-layer coating 3 is substantially constant over the entire plug. The thickness of the surface-layer coating 3 is preferably not higher than 250 pm, and more preferably not higher than 200 µm. The thickness of the surface-layer coating 3 is preferably not lower than 50 µm.

FIG. 2 is an enlarged view of portion II shown in FIG. 1. The body coating 2 and surface-layer coating 3 contain iron and iron oxides. While the body coating 2 and surface-layer coating 3 are mainly composed of iron and iron oxides, they may contain small amounts of elements and/or compounds other than iron and iron oxides. In the body coating 2, the iron content decreases and the iron-oxide content increases as it goes from the plug body 1 toward the surface-layer coating 3. The iron content in the surface-layer coating 3 is higher at least than the iron content in the region 21 of the body content 2 discussed below.

The body coating 2 includes pores. The surface-layer coating 3 also includes pores, although small and few. The porosity of the surface-layer coating 3 is lower than the porosity of the region 21 of the body coating 2. The region 21 is adjacent to the surface-layer coating 3 of the body coating 2. That is, the region 21 is a region of the body coating 2 that is located adjacent to the interface between the body coating and surface-layer coating 3. The thickness of the region 21 is substantially equal to the thickness of the surface-layer coating 3. The porosity of the surface-layer coating 3 is preferably not higher than 2.5 %. The lower the porosity of the surface-layer coating 3, the better; in practice, it is not lower than 0.5 %.

A method of calculating the iron content and iron-oxide content in and porosity of the body coating 2 and surface-layer coating 3 will be described.

First, microscopic images of cross sections of the body coating 2 and surface-layer coating 3 are obtained. In the microscopic images, the porosity of the region 21 of the body coating 2 evaluated is that of the portions of the body coating 2 that are adjacent to the interface to the surface-layer coating 3 and have the same thickness as the surface-layer coating 3. The porosity of the surface-layer coating 3 evaluated is that of the entire surface-layer coating 3 captured in the microscopic images. The area of evaluation as measured in a direction perpendicular to the thickness direction (i.e. direction parallel to the plug surface) is about 1000 to 1500 µm. Since it is assumed that pores are basically distributed homogeneously as determined in this direction, an evaluation with a width of about 1000 to 1500 µm will enable calculation of a porosity value that is substantially an average one.

FIG. 3 is an example of a microscopic image (original image) of a cross section of a coating. Iron, iron oxides and pores in the original image have their respective color tones. More specifically, the color becomes darker in the following order: iron, iron oxides, and pores.

Next, a brightness histogram is created from the original image, as shown in FIG. 4. The brightness histogram is a graph showing the pixel-brightness distribution in the original image, where the vertical axis represents frequency of occurrence (i.e. number of pixels) and the horizontal axis represents the brightness value. Detecting peaks in this brightness histogram provides three peaks derived from iron, iron oxides, and pores.

Subsequently, the original image is expressed using three values. As shown in FIG. 5, the thresholds for expression using three values are the middle value M₁ between the brightness value B₁ and brightness value B₂, and the middle value M₂ between the brightness value B2 and brightness value B₃. B₁, B₂ and B₃ are the brightness value of the peak derived from pores, the brightness value of the peak derived from iron oxides, and the brightness value of the peak derived from iron, respectively.

FIG. 6 shows a three-value image obtained by expressing the original image using three values. In the three-value image, the pixels having brightness values lower than M₁ in the original image are displayed in black, the pixels having brightness values not lower than M₁ and lower than M₂ are displayed in gray, and the pixels having brightness values not lower than M₂ are displayed in white. In the three-value image, the black regions are treated as pore regions, the gray regions as iron-oxide regions, and the white regions as iron regions, and the number of pixels in the regions of each type is counted. Dividing the number of pixels in the pore regions, the number of pixels in the iron-oxide regions, and the number of pixels in the iron regions by the total number of pixels provides the porosity (%), the content of iron oxides (%) and the content of iron (%), respectively. That is, the porosity, the content of iron oxides and the content of iron are each expressed as a value of the proportion of pixels in the original image (i.e. area ratio).

### [Method of Manufacturing Plug]

A method of manufacturing the plug 10 will be described below.

First, a plug body 1 is prepared. A body coating 2 and a surface-layer coating 3 are formed on the surface of the plug body 1 by arc spraying.

Arc spraying may be performed using, for example, arc spraying equipment 4 shown in FIG. 7. The arc spraying equipment 4 includes a spray gun 41 and a turntable 42. The spray gun 41 uses an arc to melt wire to be sprayed, and sprays it through a nozzle by means of compressed air. In the present embodiment, the wire to be sprayed is iron wire. The iron wire is wire of carbon steel (or common steel) mainly composed of iron (Fe). The iron wire is typically a so-called common steel mainly composed of Fe and including carbon (C), silicon (Si), manganese (Mn) and impurities, but may contain elements such as tungsten (W).

When the body coating 2 and surface-layer coating 3 are to be formed, the plug body 1 is placed on the turntable 42 of the arc spraying equipment 4. Then, while the turntable 42 rotates the plug body 1 about its axis, iron wire is sprayed on the plug body 1 by arc spraying. Thus, a body coating 2 containing iron and iron oxides is formed on the surface of the plug body 1. The formation of the body coating 2 is completed when a desired thickness of material is deposited on the surface of the plug body 1.

The body coating 2 is preferably formed while the spray distance is gradually increased. Spray distance refers the minimum distance between the tip of the nozzle of the spray gun 41 and the surface of the object to which spraying is done. The body coating 2 is formed by placing the spray gun 41 at a predetermined distance from the plug body 1 and initiating arc spraying, and continuing arc spraying while the spray gun 41 is gradually moved away from the plug body 1. Alternatively, the spray distance may be kept constant during the formation of the body coating 2.

Immediately after the formation of the body coating 2, a surface-layer coating 3 is formed. That is, after the body coating 2 is formed, arc spraying is continued without an interruption to form a surface-layer coating 3 on the body coating 2.

The spray distance during the formation of the surface-layer coating 3 is smaller than the spray distance during the formation of the body coating 2. More specifically, the spray distance during the formation of the surface-layer coating 3 is smaller than at least the spray distance at the completion of the formation of the body coating 2. That is, after the body coating 2 is formed while the spray gun 41 is gradually moved away from the plug body 1, the spray gun 41 is brought close to the plug body with a jerk to form the surface-layer coating 3.

While the surface-layer coating 3 is formed, the spray distance is kept substantially constant. The spray distance during the formation of the surface-layer coating 3 is preferably not larger than 200 mm. The formation of the surface-layer coating 3 is completed when a desired thickness of material is deposited on the body coating 2. Preferably, the formation of the surface-layer coating 3 is completed before the thickness of the surface-layer coating 3 exceeds 250 µm.

Spray distance will be described in more detail. FIG. 8 is a graph showing the relationship between spray distance and the porosity of a coating. FIG. 9 is a graph showing the relationship between spray distance and the content of oxides in a coating. FIG. 10 is a graph showing the relationship between spray distance and the tensile strength of a coating.

As shown in FIG. 8, the larger the spray distance, the higher the porosity of a coating becomes. That is, the porosity of the body coating 2 and surface-layer coating 3 may be controlled by adjusting the spray distance. As discussed above, the spray distance during the formation of the surface-layer coating 3 is smaller than the spray distance at the completion of the formation of the body coating 2. The porosity of the surface-layer coating 3 is lower than the porosity of the region 21 of the body coating 2.

As shown in FIG. 9, the larger the spray distance, the higher the content of oxides in a coating becomes. That is, the contents of iron and iron oxides in the body coating 2 and surface-layer coating 3 may be controlled by adjusting the spray distance. As discussed above, the body coating 2 may be formed while the spray distance is gradually increased. Thus, in the body coating 2, the iron content decreases and the iron-oxide content increases as it goes from the plug body 1 toward the surface-layer coating 3. The surface-layer coating 3 is formed by reducing the spray distance after the formation of the body coating 2. Thus, the content of iron in the surface-layer coating 3 is higher than at least the content of iron in the region 21 of the body coating 2.

As shown in FIG. 10, the larger the spray distance, the smaller the tensile strength of a coating becomes. That is, the tensile strength of the body coating 2 and surface-layer coating 3 may be controlled by adjusting the spray distance. The spray distance during the formation of the surface-layer coating 3 is smaller than the spray distance at the completion of the formation of the body coating 2. Thus, the tensile strength of the surface-layer coating 3 is larger than at least the tensile strength of the region 21 of the body coating 2.

After the body coating 2 and surface-layer coating 3 are thus formed, the plug body 1 is removed from the turntable 42 of the arc spray equipment 4. Thus, the plug 10 (FIG. 1) according to the present embodiment is finished.

### [Effects]

In the plug 10 according to the present embodiment, the surface-layer coating 3 with a low porosity is provided on the body coating 2. This prevents deformation of the body coating 2 and surface-layer coating 3 due to a load in the shear direction during piercing, thereby preventing cracks in the body coating 2 and surface-layer coating 3. These effects will be described in more detail with reference to FIGS. 11A and 11B.

FIG. 11A is a schematic cross section of portions of the plug 10 located near the surface before the piercing of a billet is initiated. As shown in FIG. 11A, the body coating 2 on the plug body 1 is covered with the surface-layer coating 3. The surface-layer coating 3 is formed by performing arc spraying of iron wire at a spray distance smaller than the spray distance at the completion of the formation of the body coating 2. Thus, the surface-layer coating 3 has a porosity lower than the porosity of the region of the body coating 2 located adjacent to the surface-layer coating 3, and is dense and has a high tensile strength.

FIG. 11B is a schematic cross section of portions of the plug 10 located near the surface during the piercing of a billet. As shown in FIG. 11B, when the piercing of the billet is initiated, a load in the shear direction acts on the surface of the surface-layer coating 3. However, the surface-layer coating 3 is dense and has a high tensile strength, and thus cannot easily be deformed by the load in the shear direction. The body coating 2 cannot easily be deformed, either, since it is covered with the surface-layer coating 3. Thus, in the body coating 2 and surface-layer coating 3, no crack occurs that would lead to a peel-off. Thus, the body coating 2 and surface-layer coating 3 are prevented from peeling off.

The body coating 2 and surface-layer coating 3 can be easily formed by arc spraying using iron wire. Further, the body coating 2 and surface-layer coating 3 are successively formed within one and the same step. Thus, the present embodiment will allow a plug 10 with a coating having a high peeling resistance to be manufactured in a simple manner.

The porosity of the surface-layer coating 3 is preferably not higher than 2.5 %. Thus, the surface-layer coating 3 is denser, providing sufficient tensile strength of the surface-layer coating 3. This will effectively prevent deformation of and cracks in the body coating 2 and surface-layer coating 3. This will prevent peel-off of the body coating 2 and surface-layer coating 3 more reliably. As discussed above, the lower the porosity of the surface-layer coating 3, the better; in practice, it is not lower than 0.5 %.

The thickness of the surface-layer coating 3 is preferably not higher than 250 µm. This will prevent the temperature of the surface-layer coating 3 from rising during piercing/rolling. As discussed above, the surface-layer coating 3 has a high iron content in the coating, and thus has a high heat conductivity. Thus, the surface-layer coating 3 can easily be heated as it contacts a hot billet during piercing/rolling. If the thickness of the surface-layer coating 3 is too large, heat can be accumulated within the surface-layer coating 3, leading to high temperatures in the surface-layer coating 3. If the surface-layer coating 3 is too hot, the billet can easily seize on the plug 10. A thickness of the surface-layer coating 3 that is not larger than 250 µm will prevent seizure.

The thickness of the surface-layer coating 3 is preferably not smaller than 50 µm. This will prevent the body coating 2 and surface-layer coating 3 from deforming due to the load in the shear direction during piercing, thereby preventing cracks more reliably.

The body coating 2 is formed while the spray distance is gradually increased. Thus, the iron content is high in a region of the body coating 2 that is adjacent to the plug body 1, thereby improving the adhesion between the plug body 1 and body coating 2. On the other hand, the iron-oxide content is high in a region of the body coating 2 that is adjacent to the surface-layer coating 2, and thus the heat conductivity is low, thereby improving heat insulation. This will prevent the billet from seizing on the plug 10.

While embodiments have been described, the present disclosure is not limited to the above-described embodiments, and various modifications are possible without departing from the spirit of the invention.

### EXAMPLES

The present disclosure will be described in more detail below with reference to examples. The present disclosure is not limited to the examples below.

Six steel plug bodies (1) with a maximum diameter of 77.5 mm, with a total length of 230 mm, and containing 0.15 mass % C and 3.5 mass % W were prepared. Arc spraying using iron wire formed a body coating (2) on the surface of each plug body (1). During the formation of the body coating (2), spraying was performed while the spray distance was changed from 200 mm to 1000 mm. The thickness of the body coating (2) was 1200 µm as measured at the tip (11) of the plug body (1) and 500 µm as measured at the trunk portion (12).

For five plug bodies (1), a surface-layer coating (3) was formed on the body coating (2) by arc spraying using iron wire to provide plugs according to Inventive Examples 1 to 5. The conditions for forming the surface-layer coating (3) are shown in Table 1. For the remaining one plug body (1), no surface-layer coating (3) was provided, and this provided a plug according to a Comparative Example.

**[Table 1]**

| | Work conditions | | | Results | |
|---|---|---|---|---|---|
| | Spray conditions and coating thickness | Proportion of pores in coating | | Life pass number | Peeling of coating on trunk |
| | Surface-layer coating | Body coating *1 | Surface-layer coating | | |
| Comp. Ex. | none | 13.8 | - | 3 | poor |
| Inv. Ex. 1 | spray distance: 100 mm 300 *µ* m thick | 9.3 | 1.7 | 1 | good |
| Inv. Ex. 2 | spray distance: 300 mm 100 *µ* m thick | 13.8 | 2.7 | 4 | acceptable |
| Inv. Ex. 3 | spray distance: 100 mm 100 *µ*m thick | 13.8 | 1.7 | 7 | good |
| Inv. Ex. 4 | spray distance: 100 mm 200 *µ* m thick | 11.3 | 1.7 | 8 | good |
| Inv. Ex. 5 | spray distance: 200 mm 200 *µ*m thick | 11.3 | 2.2 | 8 | good |

| | | | | | |
|---|---|---|---|---|---|
| *1 The porosity of the body coating evaluated was that of the region adjacent to the surface layer (i.e. interface between the body coating and surface-layer coating) and having the same thickness as the surface-layer coating. The value of the comparative example is the value for the region of 100 µm adjacent to the surface. | | | | | |

The plugs according to Inventive Examples 1 to 5 and the Comparative Example were repeatedly used to perform piercing/rolling on billets made of SUS 304 with a diameter of 65 mm and a length of 400 mm that had been heated to 1200 °C. For each of Inventive Examples 1 to 5 and the Comparative Example, the number of piercing rounds performed until the plug was damaged (i.e. life pass number), and how damaged the plug was, were determined. The life pass numbers and how damaged the plugs were for Inventive Examples 1 to 5 and the Comparative Example are shown in Table 1.

In the plug of the Comparative Example, the coating peeled off the trunk portion (12) during the third pass. In contrast, in Inventive Examples 3 to 5, the coating did not peel off even after seven or eight passes. In Inventive Example 1, seizure occurred during the first pass and piercing rolling was halted at this point, where the coating did not peel off the trunk portion (12). In Inventive Example 2, the coating peeled off the trunk portion (12) during the fourth pass. This demonstrates that providing a surface-layer coating (3) on the body coating (2) prevents peeling of the coating. In each of Inventive Examples 3 to 5, the deformation of the plug tip (11) after the life pass number listed in Table 1 exceeded a permitted range, and the piercing/rolling was halted at this point.

In Inventive Example 1, the thickness of the surface-layer coating (3) was 300 pm, which is larger than 250 µm. In Inventive Example 1, the billet seized on the plug during the first pass. In contrast, in each of Inventive Examples 2 to 5, where the thickness of the surface-layer coating (3) was not larger than 250 pm, the billet did not seize on the plug. Thus, the thickness of the surface-layer coating (3) is preferably not larger than 250 µm to prevent seizure.

In each of Inventive Examples 1 and 3 to 5, the porosity of the surface-layer coating (3) was not higher than 2.5 %, meaning that the density and strength of the surface-layer coating (3) were high. Consequently, in each of Inventive Examples 1 and 3 to 5, the coating did not peel off. On the other hand, in Inventive Example 2, the spray distance during the formation of the surface-layer coating (3) was 300 mm and the porosity of the surface-layer coating (3) was 2.7 %. That is, the density and strength of the surface-layer coating (3) in Inventive Example 2 were lower than in Inventive Examples 1 and 3 to 5. Consequently, the coating of Inventive Example 2 peeled off during the fourth pass. These results show that the porosity of the surface-layer coating (3) is preferably not higher than 2.5 % to prevent peeling of the coating more effectively.

## Claims

1. A plug used for piercing a billet, comprising:
a plug body (1);
a body coating (2) provided on a surface of the plug body (1) and containing iron and iron oxides; and
a surface-layer coating (3) provided on the body coating (2) and containing iron and iron oxides,
wherein the surface-layer coating (3) has a porosity lower than that of a region of the body coating (2) adjacent to the surface-layer coating (3), the region having a thickness equal to that of the surface-layer coating (3),
the body coating (2) has an iron content which decreases and an iron oxide content which increases from the plug body (1) toward the surface layer coating (3), **characterized in that**
the surface-layer coating (3) has an iron content higher than the region of the body coating (2) adjacent to the surface-layer coating (3) and having a thickness equal to that of the surface-layer coating (3).

2. The plug according to claim 1, wherein the porosity of the surface-layer coating (3) is not higher than 2.5 %.

3. The plug according to claim 1 or 2, wherein the thickness of the surface-layer coating (3) is not larger than 250 µm.

4. The plug according to any one of claims 1 to 3, wherein the body coating (2) covers an entire surface of the plug body (1) except for a rear end surface of the plug body (1).

5. The plug according to any one of claims 1 to 4, wherein the body coating (2) has a thickness which is not constant.

6. The plug according to any one of claims 1 to 5, wherein the surface-layer coating (3) covers an entire surface of the body coating (2).

7. The plug according to any one of claims 1 to 6, wherein the surface-layer coating (3) has a thickness not lower than 50 µm.

8. A method of manufacturing a plug used for piercing a billet according to any one of claims 1 to 7, comprising:
preparing a plug body (1);
forming a body coating (2) on a surface of the plug body (1) by performing arc spraying using iron wire; and
forming a surface-layer coating (3) on the body coating (2) by performing arc spraying using iron wire at a spray distance shorter than that at completion of the formation of the body coating (2).

9. The method of manufacturing a plug according to claim 8, wherein in the forming of the body coating (2), arc spraying is performed while the spray distance is gradually increased.

10. The method of manufacturing a plug according to claim 9, wherein after the body coating (2) is formed by a spray gun, the spray gun is brought close to the plug body (1) with a jerk to form the surface layer coating (3).

11. The method of manufacturing a plug according to any one of claims 8 to 10, wherein formation of the surface-layer coating (3) is completed before a thickness of the coating exceeds 250 µm.

## Patentansprüche

1. Ein Stechdorn, der zum Durchstechen eines Knüppels verwendet wird, umfassend:
einen Stechdornkörper (1);
eine Körperbeschichtung (2), die auf einer Oberfläche des Stechdomkörpers (1) vorgesehen ist und Eisen und Eisenoxide enthält; und
eine Oberflächenschichtbeschichtung (3), die auf der Körperbeschichtung (2) vorgesehen ist und Eisen und Eisenoxide enthält,
wobei die Oberflächenschichtbeschichtung (3) eine geringere Porosität aufweist als die eines Bereichs der Körperbeschichtung (2), welcher an die Oberflächenschichtbeschichtung (3) angrenzt, wobei der Bereich eine Dicke aufweist, die gleich der der Oberflächenschichtbeschichtung (3) ist,
wobei die Körperbeschichtung (2) einen vom Stechdornkörper (1) hin zu der Oberflächenschichtbeschichtung (3) abnehmenden Eisengehalt und einen zunehmenden Eisenoxidgehalt aufweist, **dadurch gekennzeichnet, dass**
die Oberflächenschichtbeschichtung (3) einen höheren Eisengehalt aufweist als der Bereich der Körperbeschichtung (2), der an die Oberflächenschichtbeschichtung (3) angrenzt und eine Dicke hat, die gleich der der Oberflächenschichtbeschichtung (3) ist.

2. Stechdorn nach Anspruch 1, wobei die Porosität der Oberflächenschichtbeschichtung (3) nicht höher als 2,5 % ist.

3. Stechdorn nach Anspruch 1 oder 2, wobei die Dicke der Oberflächenschichtbeschichtung (3) nicht größer als 250 µm ist.

4. Stechdorn nach einem der Ansprüche 1 bis 3, wobei die Körperbeschichtung (2) eine gesamte Oberfläche des Stechdornkörpers (1) mit Ausnahme einer hinteren Endfläche des Stechdomkörpers (1) bedeckt.

5. Stechdorn nach einem der Ansprüche 1 bis 4, wobei die Körperbeschichtung (2) eine Dicke aufweist, die nicht konstant ist.

6. Stechdorn nach einem der Ansprüche 1 bis 5, wobei die Oberflächenschichtbeschichtung (3) eine gesamte Oberfläche der Körperbeschichtung (2) bedeckt.

7. Stechdorn nach einem der Ansprüche 1 bis 6, wobei die Oberflächenschichtbeschichtung (3) eine Dicke von nicht weniger als 50 µm aufweist.

8. Verfahren zur Herstellung eines Stechdoms, der zum Durchstechen eines Knüppels verwendet wird, nach einem der Ansprüche 1 bis 7, umfassend:
Vorbereitung eines Stechdomkörpers (1);
Ausbilden einer Körperbeschichtung (2) auf einer Oberfläche des Stechdomkörpers (1) durch Ausführen eines Lichtbogenspritzens unter Verwendung von Eisendraht; und
Ausbilden einer Oberflächenschichtbeschichtung (3) auf der Körperbeschichtung (2) durch Ausführen von Lichtbogenspritzen unter Verwendung von Eisendraht in einem Sprühabstand, der kürzer ist als derjenige bei Abschluss der Ausbildung der Körperbeschichtung (2).

9. Verfahren zur Herstellung eines Stechdoms nach Anspruch 8, wobei bei der Bildung der Körperbeschichtung (2) ein Lichtbogenspritzen durchgeführt wird, während der Sprühabstand graduell vergrößert wird.

10. Verfahren zur Herstellung eines Stechdoms nach Anspruch 9, wobei nach dem Ausbilden der Körperbeschichtung (2) durch eine Spritzpistole die Spritzpistole mit einem Ruck an den Stechdornkörper (1) herangeführt wird, um die Oberflächenschichtbeschichtung (3) zu bilden.

11. Verfahren zur Herstellung eines Stechdoms nach einem der Ansprüche 8 bis 10, wobei die Bildung der Oberflächenschichtbeschichtung (3) abgeschlossen wird, bevor eine Dicke der Beschichtung 250 µm überschreitet.

## Revendications

1. Poinçon utilisé pour percer une billette, comprenant :
un corps de poinçon (1) ;
un revêtement de corps (2) fourni sur une surface du corps de poinçon (1) et contenant du fer et des oxydes de fer ; et
un revêtement de couche de surface (3) fourni sur le revêtement de corps (2) et contenant du fer et des oxydes de fer,
dans lequel le revêtement de couche de surface (3) présente une porosité inférieure à celle d'une région du revêtement de corps (2) adjacente au revêtement de couche de surface (3), la région ayant une épaisseur égale à celle du revêtement de couche de surface (3),
le revêtement de corps (2) présente une teneur en fer qui diminue et une teneur en oxyde de fer qui augmente à partir du corps de poinçon (1) vers le revêtement de couche de surface (3), **caractérisé en ce que**
le revêtement de couche de surface (3) présente une teneur en fer supérieure à la région du revêtement de corps (2) adjacente au revêtement de couche de surface (3) et ayant une épaisseur égale à celle du revêtement de couche de surface (3).

2. Poinçon selon la revendication 1, dans lequel la porosité du revêtement de couche de surface (3) n'est pas supérieure à 2,5 %.

3. Poinçon selon la revendication 1 ou 2, dans lequel l'épaisseur du revêtement de couche de surface (3) n'est pas plus large que 250 µm.

4. Poinçon selon l'une quelconque des revendications 1 à 3, dans lequel le revêtement de corps (2) recouvre une surface entière du corps de poinçon (1) à l'exception d'une surface d'extrémité arrière du corps de poinçon (1).

5. Poinçon selon l'une quelconque des revendications 1 à 4, dans lequel le revêtement de corps (2) présente une épaisseur qui n'est pas constante.

6. Poinçon selon l'une quelconque des revendications 1 à 5, dans lequel le revêtement de couche de surface (3) recouvre une surface entière du revêtement de corps (2).

7. Poinçon selon l'une quelconque des revendications 1 à 6, dans lequel le revêtement de couche de surface (3) présente une épaisseur d'au moins 50 µm.

8. Procédé de fabrication d'un poinçon utilisé pour percer une billette selon l'une quelconque des revendications 1 à 7, comprenant :
la préparation d'un corps de poinçon (1) ;
la formation d'un revêtement de corps (2) sur une surface du corps de poinçon (1) en réalisant une pulvérisation à l'arc utilisant un câble en fer ; et
la formation d'un revêtement de couche de surface (3) sur le revêtement de corps (2) en réalisant une pulvérisation à l'arc en utilisant un câble de fer à une distance de pulvérisation plus courte qu'à l'achèvement de la formation du revêtement de corps (2).

9. Procédé de fabrication d'un poinçon selon la revendication 8, dans lequel dans la formation du revêtement de corps (2), une pulvérisation à l'arc est réalisée alors que la distance de pulvérisation est progressivement augmentée.

10. Procédé de fabrication d'un poinçon selon la revendication 9, dans lequel après que le revêtement de corps (2) est formé par un pistolet de pulvérisation, le pistolet de pulvérisation est amené à proximité du corps de poinçon (1) avec une secousse pour former le revêtement de couche de surface (3).

11. Procédé de fabrication d'un poinçon selon l'une quelconque des revendications 8 à 10, dans lequel la formation du revêtement de couche de surface (3) est achevée avant qu'une épaisseur du revêtement excède 250 µm.
